

# UNITED STATES PATENT OFFICE.

MARINUS RAPPARD, OF DEN HELDER, NETHERLANDS.

## MANUFACTURE OF PAINT FOR PROTECTING IRON, WOOD, AND THE LIKE FROM SEA GROWTHS.

1,108,395.

Specification of Letters Patent. Patented Aug. 25, 1914.

No Drawing.

Application filed October 7, 1912. Serial No. 724,431.

To all whom it may concern:

Be it known that I, MARINUS RAPPARD, subject of the Queen of the Netherlands, residing at Den Helder, Kingdom of the Netherlands, have invented certain new and useful Improvements in the Manufacture of Paint for Protecting Iron, Wood, and the like from Sea Growths, of which the following is a specification.

10 The present invention relates to the manufacture of a paint to be applied to iron, wooden or the like surfaces, to protect them from the destructive action of sea-growths.

15 Of all known coatings or coverings the only one which affords any real protection against sea growths is a coating of plates of copper and wooden vessels have been so protected with great success, the plates having remained efficient for many years. Red 20 copper plates have also been applied to iron vessels, but in order to prevent the galvanic action arising between the iron of the ship's skin and the copper and to enable the plates to be properly attached a layer of insulating 25 material had first to be applied to which the copper plates could be readily attached. This method, however, was very expensive and is no longer used and reliance is placed solely upon paints for protecting iron ships.

30 The paints which have hitherto been used lose their power after a short time, so that the ships have to be re-coated at regular intervals after the removal of any growths which may have accumulated and this also 35 is expensive. It has also been proposed to prepare paints of an alloy of copper with another metal or other metals in a finely divided form mixed with a suitable fluid medium, or to spread or distribute pulverized 40 copper, or an alloy thereof, on an anti-fouling paint before the latter has become hardened or set. The copper powder is sometimes mixed with anti-fouling paint (lead-paint) before being applied to the ship's

45 hull, either with or without the subsequent application of pulverized copper or an alloy thereof. Another paint for preventing the fouling of ships' bottoms or the like, is prepared by mixing pulverized copper with 50 pulverized red lead and incorporating this mixture in a vehicle consisting of a solution of caoutchouc in oil or turpentine or other suitable solvent, boiled linseed oil and common rosin. It has also been proposed to

suspend zinc in a semi-saturated solution of 55 sulfate of copper and to mix the deposit after pulverization, with Chinese varnish, or to mix finely divided metallic copper or an alloy thereof with a vehicle derived from the sludge oil resulting from the refining of 60 petroleum.

According to the present invention a paint is manufactured which is intended to form a coating of copper on the ship's skin in such a manner that it has the same properties with respect to sea growths as the red copper plates have, and at the same time prevents the galvanic action between the ship's skin and the copper coating. This paint consists mainly of copper in finely 65 powdered form mixed in suitable proportions with shellac in combination with oil (preferably linseed oil), this combination being most suitable owing to its high binding power and insulating qualities and also 70 the rapidity with which it dries in the air. The copper powder may be made from pure copper or from an alloy containing a high percentage of copper.

The paint may be made in any suitable 80 manner, for instance by first dissolving the shellac in alcohol, and then adding the copper and oil while the mixture is continuously stirred. Suitable mixtures contain 3-6 parts by weight of copper powder, 1-2.5 85 parts of dry shellac dissolved in 3-7 parts of alcohol and 3.5-8.75 parts of oil. If the paint is made in this way each particle of the copper receives a coating of shellac and oil, so that on applying the paint to the surface of the ship an insulating layer between the latter and the copper is formed, while the protective action of the copper against 90 sea-growths is not affected by the shellac and oil.

To enhance the insulating effect a coating of zinc or a zinc compound and oil or shellac may first of all be applied to the usual coating of red lead paint and the new paint applied directly to this zinc coating. Experiments have shown, however, that the shellac and oil sufficiently insulate the copper from the iron of the ship's hull. The hull may therefore be merely painted with red lead paint in the usual manner for protection 100 from rust and the copper paint then applied; a single coat of the latter suffices 105 whereas all the other paints require to be

applied at least twice, which alone constitutes a considerable saving. The painted surface is very smooth and affords little foothold for algæ and the like, which is 5 not the case with other paints.

By painting ships, boats, pontoons and the like with the new paint, the growth of sea-plants and sea-animals is entirely prevented by the action of the copper.

10 What I claim is:

1. The herein described paint for iron, wood, and the like, comprising 3-6 parts of finely divided metal containing copper, 1-2.5 parts of dry shellac dissolved in 3-7

parts of alcohol, and 3.5-8.75 parts of a 15 siccative oil.

2. A paint containing finely-divided metal containing a high percentage of copper, mixed and suspended in an alcoholic solution of shellac and a siccative oil. 20

In testimony whereof I have hereunto set my hand in presence of two subscribing witnesses.

MARINUS RAPPARD.

Witnesses:

W. DE MAAN,  
F. W. DAENDELS.